

# UNITED STATES PATENT OFFICE.

FREDERIC E. CARTER, OF NEWARK, NEW JERSEY, ASSIGNOR TO BAKER & COMPANY, INC., A CORPORATION OF NEW JERSEY.

## ALLOY.

1,357,272.

Specification of Letters Patent.

Patented Nov. 2, 1920.

No Drawing.

Application filed January 20, 1920. Serial No. 352,873.

To all whom it may concern:

Be it known that I, FREDERIC EDWARD CARTER, a subject of Great Britain, and a resident of Newark, in the county of Essex and State of New Jersey, have invented new and useful Improvements in Alloys, of which the following is a specification.

This invention relates more particularly to an alloy to replace platinum-iridium, as it is employed for hypodermic needles, magneto contacts and the like, and the objects of the invention are to avoid the use of iridium, which is expensive and difficult to obtain; to obtain an alloy which shall closely simulate platinum-iridium in all the qualities which render it especially adapted to the uses for which it is employed; to obtain a practicable facility in working the alloy, and to obtain other advantages and results as may be brought out in the following description.

In carrying out my invention I form an alloy of gold, silver and palladium with an excess of platinum, and while other proportions may be useful in other arts, the proportions for a substitute for platinum-iridium should be substantially 5%-15% of gold,  $\frac{1}{2}\%-5\%$  of silver and  $\frac{1}{2}\%-5\%$  of palladium, the rest of the alloy being platinum.

It will be understood that the proportions of the metals can be varied to make the alloy more or less workable and soft, for different purposes or uses, as for example, the particular proportions which I have employed in an alloy for magneto contacts are gold 12.3%, silver 1.8%, palladium 1.3% and platinum 84.6%.

The excess of platinum, in my new alloy, enables the desired qualities of platinum-iridium to be obtained without the use of any iridium, and, while of course the platinum is expensive, an alloy is obtained which because of the absence of the still more expensive iridium is more economical than platinum-iridium. In this way a less expensive substitute for platinum-iridium is secured and the supply of iridium conserved.

Having thus described the invention, what I claim is:

1. An alloy containing substantially 5%-15% gold,  $\frac{1}{2}\%-5\%$  silver,  $\frac{1}{2}\%-5\%$  palladium and the rest platinum.
2. An alloy containing 12.3% gold, 1.8% silver, 1.3% palladium and 84.6% platinum.

FRED. E. CARTER.